

Sept. 26, 1967

H. W. GOODNER

3,343,753

YARN WINDING PROCESS AND PRODUCT

Filed March 5, 1965



INVENTOR  
H. W. GOODNER

BY

*Stanley M. Tarter*  
ATTORNEY

1

3,343,753  
YARN WINDING PROCESS AND PRODUCT  
Homer W. Goodner, Pensacola, Fla., assignor to  
Monsanto Company, St. Louis, Mo., a corporation  
of Delaware  
Filed Mar. 5, 1965, Ser. No. 437,473  
8 Claims. (Cl. 242—18)

## ABSTRACT OF THE DISCLOSURE

A yarn winding process and package of yarn of at least 840 denier wound on small diameter bobbins with a 6-inch traverse stroke and a winding ratio of bobbin revolutions to traverse cycles in the range of 3.354125:1 to 3.412500:1.

The term "heavy denier yarn" and "industrial yarn" as used herein applies to yarn having a count of approximately 840 total denier and above. Nylon yarns of 840 denier are used in tire cord production and are an example of industrial yarn. Conventionally, large diameter packages of heavy denier yarn have not been packaged on small diameter yarn holders, i.e., bobbins, pirns, tubes and cones. Early efforts made to wind large packages of heavy denier yarns on small yarn holders using short traverse strokes of approximately six (6) inches and employing known wind ratios were unsuccessful. Suggested wind ratios of bobbin revolutions to traverse cycles per minute such as 3:1 and 4:1 were tried. The packages formed using the known wind ratios were unacceptable and below standard due to pronounced sloughing of the wraps. The problem was particularly difficult in winding so-called flat yarn or yarn having substantially no twist imparted therein. It has been discovered that heavy denier yarns, including flat yarns and yarns having low friction finishes applied thereon, can be successfully wound to form stable, acceptable yarn packages if a specific new and critical decimal winding ratio range is used.

For purposes of illustration, the process and package embodying the invention will be described as carried out on a cone winding machine. It will be understood that other winding apparatus may be used and that the yarn holder need not be a cone but can be a straight tube. In cone winding, a constant ratio of bobbin or spindle revolution (r.p.m.) to yarn traversal rate measured in cycles per minute (c.p.m.) is maintained throughout the packaging operation. A selected ratio of spindle r.p.m. to traversal c.p.m. may be provided by a conventional gear-gainer mechanism. Success in winding an acceptable and stable yarn package of heavy denier yarn on relatively small diameter cones was achieved employing a critical decimal ratio of spindle r.p.m. to traverse c.p.m. The phrase "traverse cycle" or a "yarn traversal" as used herein comprises one back and forth displacement of yarn on a bobbin or package circumference or circumferences.

The object of this invention is to form yarn packages of heavy industrial deniers, particularly those with little or no twist referred to as "flat" yarns, on small diameter yarn holders employing a critical winding ratio.

According to the invention, stable packages of heavy denier yarn are formed on small diameter bobbins (two inches or less outer diameter for straight or uniform diameter tubes and two inches or less mean outer diameter for cones) using a constant ratio of spindle or bobbin r.p.m. to traverse c.p.m. in the range of 3.354125:1 to 3.412500:1.

A better understanding of the invention will be gained by reference to the following description and to the single figure in the accompanying drawing.

The process and product embodying the invention are

2

illustrated in the drawing in conjunction with a coning machine known as a coner 1. Only the essential features of the coner 1 are shown. Coner 1 includes a spindle 2 driven by motor means 3. A bobbin 4 is mounted on spindle 2 and a traverse guide 5 is positioned adjacent the bobbin. Traverse guide 5 is operatively connected to motor means 3 and adapted for reciprocation back and forth axially of the bobbin. The ratio of spindle r.p.m. to traverse c.p.m. is selectable through an interconnecting gear train 6. A pivoted pressure roller 7 surfacey engages the yarn package being formed, and an adjustable tension device 8 provides a desired tension.

Several examples of successful packaging of heavy denier yarns on small bobbins are given below.

### Example I

According to this example, packages of eight (8) pound weight were formed of filament yarn having a total denier count of 840 on standard cone bobbins having a 3°30' taper, a 7/4 inches length and an outer diameter of approximately two inches at the base thereof. The diameter of the package formed was approximately 9 1/2 inches at the base of the cone. Coner 1 was equipped with a gear train to furnish a ratio of spindle or bobbin r.p.m. to traverse c.p.m. of 3.354125 to 1. The traverse stroke used was approximately 6 inches. Industrial heavy denier yarn of 840 total denier and 140 filaments was unwound from a supply "cake" 9 and laced into the traverse guide 5 and about cone 4. Coner 1 was then operated. Stable, commercially acceptable yarn packages were produced. The yarn wraps on the packages tightly interlocked and did not slough. In forming packages, yarn winding tension was maintained at from 40-45 gms. at start-up and was continually and smoothly decreased to a tension of 18-23 gms. at the end of package formation. Roller 7 pressure at start-up was from 600-800 gms. and was continually and smoothly decreased to 100-200 gms. at the finish.

### Example II

Acceptable, stable packages of eight (8) pound yarn packages of heavy denier yarn were formed employing operating conditions similar to those given in Example I with the exception that the packages were wound with a ratio of spindle speed to traverse cycles of 3.412500:1 and with only slight variation in winding tension and roller pressure.

### Example III

Acceptable, stable packages of five (5) and ten (10) pound weight of heavy denier yarn were also formed employing the same coner referred to in Examples I and II and operating in the range of spindle revolutions to traverse cycle speed of 3.354125:1 and 3.412500:1.

The examples given above relate to cone winding, however, the winding operation can be performed on small straight tubes and bobbins. The critical features that provide a successful winding of yarn packages are the decimal winding ratio range provided, the yarn count, the bobbin size and the traverse stroke used. The tensions and forces of the pressure roll used are within known limits and are not critical.

It will be understood that variations and modifications of the invention are contemplated within the spirit thereof and the scope of the following claims.

I claim:

1. A filament yarn winding process comprising, delivering yarn having a total denier count of at least 840 to a winding and traversing zone, winding said filament yarn on a driven tubular bobbin, traversing said filament yarn with approximately a 6-inch traverse stroke across said tubular bobbin, maintaining a winding ratio of bobbin revolutions

to traverse cycles in the range of 3.354125:1 to 3.412500:1, inclusive, while packaging said filament yarn on said tubular bobbin.

2. A filament yarn winding process as in claim 1, wherein said filament yarn is wound on a straight tubular bobbin having an outer diameter of two inches or less.

3. A filament yarn winding process as in claim 1, wherein said filament yarn is wound on a cone bobbin having a 3°30' taper and an outer diameter of two inches or less at the base thereof.

4. A filament yarn winding process as in claim 1, wherein said filament yarn is wound on a cone bobbin having a 3°30' taper and a mean outer diameter of two inches or less.

5. A filament yarn package comprising, 15 convolutions of filament yarn having a total denier of at least 840 wound on a tubular bobbin, said filament yarn being spread across approximately 6 inches of the face of said tubular bobbin, said filament yarn being wound wherein the number of 20 wraps taken around the circumference of said pack-

age as related to each back and forth traversal of said filament yarn across said package is within the winding ratio range of 3.354125:1 to 3.412500:1.

6. A filament yarn package as in claim 5, wherein 5 said filament yarn is wound on a straight tubular bobbin having an outer diameter of two inches or less.

7. A filament yarn package as in claim 5, wherein said filament yarn is wound on a cone bobbin having a 3°30' taper and an outer diameter of approximately two inches or less at the base thereof.

10 8. A filament yarn package as in claim 5, wherein said filament yarn is wound on a cone bobbin having a 3°30' taper and a mean outer diameter of two inches or less.

#### References Cited

##### UNITED STATES PATENTS

|           |        |                 |       |         |
|-----------|--------|-----------------|-------|---------|
| 2,649,254 | 8/1953 | Balthrop        | ----- | 242—43  |
| 2,764,368 | 9/1956 | Halkyard et al. | ----- | 242—177 |
| 3,193,209 | 7/1965 | Hambach         | ----- | 242—18  |

20 STANLEY N. GILREATH, Primary Examiner.